

## UNITED STATES PATENT OFFICE

2,276,415

PROCESS OF PRODUCING COATED FABRICS  
AND PRODUCT THEREOF

Alan E. Murray, Wilmington, Del.

No Drawing. Application October 31, 1938,  
Serial No. 237,887

6 Claims. (Cl. 91—68)

My invention relates particularly to a process and product thereof, whereby fabrics of all kinds may be treated in an advantageous way and having novel properties.

The object of my invention is to provide a process and product whereby fabrics may be obtained of an advantageous character. The object is, furthermore, to provide fabrics having novel properties and which have characteristics not hitherto attained. The object is, furthermore, particularly to obtain fabrics, no matter how rough and uneven the surface may be, which are, in accordance with my invention, provided with a coating, which may be extremely thin, of rubber whereby the fabrics obtained may retain substantially their original appearance and yet be washable so as to wash foreign materials, such as dirt, from the surface of the same. Another object is to provide such fabrics whereby, if desired, notwithstanding the coating of rubber, fibres of the fabric may extend through the rubber coating and above the surface thereof so as to aid in retaining the original appearance and general characteristics of the fabric notwithstanding the coating of rubber thereon or therein. Another object is to provide such a coating which is securely anchored and inseparably bonded to the fabric so as to withstand wear to an extraordinary extent. Further objects of my invention will appear from the detailed description of the same hereinafter.

While my invention is capable of embodiment in many different forms, for the purpose of illustration I have described in detail hereinafter only certain embodiments of the same.

For example, I may proceed as follows in accordance with my invention: Any desired type of fabric made out of fibres, but, for example, a woven fabric as for instance of cotton, linen, or wool, but preferably cotton, and which may have a surface of extraordinary unevenness, if desired, is first dusted over with a dust of any desired substantially inert material. For this purpose I prefer to use as one such inert material a dust of plaster of Paris, and particularly the material known in the trade as Hydrocal, which is a very highly dehydrated plaster of Paris ground to an extreme fineness. For this purpose any other kind of inert dust may be used for a part or all of the plaster of Paris, if deemed desirable, however, for instance kieselguhr or cotton flock powder or lycopodium powder or colloidal clays. The dust is then largely shaken off or dusted off, as, for example, by slightly rubbing or beating two dusted surfaces of the fabric together. This

leaves a slightly white cast to the dusted surface in the case where white powder has been used. This dustiness of the surface of the fabric prevents the penetration of the coating given as hereinafter described, and in the case of the plaster of Paris dust combines with the water present in the coating material due to the extraction of water from the latter by the plaster of Paris and becoming combined with the plaster of Paris as water of crystallization in the setting thereof. The surface of the fibre having been thus prepared with the dusting material, I apply a coating of any desired type of latex, that is to say any rubber material carried in water suspension, as, for example, any of the latex materials set forth in the patents to Philip Schidrowitz, Nos. 1,443,149, 1,682,857 and 1,939,635, but I preferably use what is known as a pre-vulcanized latex known under the name of "Vultex" for this purpose and which has a strong ammonia odor. This latex material is preferably applied in dilute form, that is to say containing one part by volume of the latex and four parts by volume of the water. The water used for this purpose should be preferably distilled water or at least water without any chlorine content, as the latter would tend to coagulate the contents. The latex material is applied to the fabric in any desired way, as, for instance, by wiping the same over the surface or spraying it thereon until a thin coating has thus been applied. It will be found that owing to the presence of the dust the liquid will not penetrate beneath the superficial portion of the fabric to any appreciable extent. When the material has dried, by the evaporation of the water therefrom, it will be found that the fabric has received an extremely thin protective coating of the latex or rubber without materially changing the surface appearance of the fabric. Where the fabric has, for instance, a dull or matt surface this same appearance will be found to be retained. If it is desired to produce a fabric having the superficial fibres or fuzz projecting from the surface of the fabric, this can be done by applying or rubbing a wash over the surface of the fabric while the surface of the fabric is still wet with the coating material as above-described. In other words, this wash can be applied before the coating material has been allowed to dry to any extent or it can be applied after the coating material has been partially allowed to dry. The wash used for this purpose is comprised preferably of one part by volume of the same undiluted latex used as previously described, diluted with twenty parts by volume of water. After this

washing has been accomplished and the fabric has been allowed to dry, it will be found that the superficial fibres of the fabric project outwardly from the rubber coating, preserving in minute detail the original appearance of the fabric. 5

The fabrics so obtained are washable and any dirt or foreign material can be readily removed therefrom by merely rubbing a damp cloth over the surface thereof, also they are waterproof and yet when a thin coating has been thus applied it has been found that the fabric is still somewhat porous, the porosity being relative to the thickness of the coating applied. These fabrics are particularly desirable as decorative fabrics, 10 wall fabrics, etc.

This type of procedure can also be applied to paper instead of the fabrics above specified.

Furthermore, any of the above fabrics, such, for example, as woven cotton, linen or wool or paper, can, after being coated as above with the powder and then the latex, and before the final drying of the latter, be effectively bonded to leather in that condition because of the superficial position of the latex, which otherwise would so penetrate 25 the fabric as not to be available for effective bonding of the fabric to the leather.

While I have described my invention above in detail I wish it to be understood that many changes may be made therein without departing 30 from the spirit of the same.

I claim:

1. The process which comprises applying to a fabric a coating of a substantially inert dust, then applying thereto an aqueous suspension of rubber, then washing off a part of the aqueous suspension of rubber to leave only a thin film on the fibres leaving the mesh open and the nap relatively uncoated, and drying the fabric so that in the finished product the said fibres are covered with only a thin rubber film leaving the mesh open. 35

2. The process which comprises applying to a fabric a coating of dust of plaster of Paris, then applying thereto an aqueous suspension of rubber, then washing off a part of the aqueous suspension of rubber to leave only a thin film on the fibres leaving the mesh open and the nap rela- 40

tively uncoated, and drying the fabric so that in the finished product the said fibres are covered with only a thin rubber film leaving the mesh open.

3. The process which comprises applying to a fabric a coating of substantially inert dust, then applying thereto an aqueous suspension of rubber, then washing off a part of the aqueous suspension of rubber with the same aqueous suspension of rubber but diluted with water to leave only a thin film on the fibres leaving the mesh open and the nap relatively uncoated, and drying the fabric so that in the finished product the said fibres are covered with only a thin rubber film leaving the mesh open.

4. The process which comprises applying to a fabric a coating of dust of plaster of Paris, then applying thereto an aqueous suspension of rubber, then washing off a part of the aqueous suspension of rubber with the same aqueous suspension of rubber but diluted with water to leave only a thin film on the fibres leaving the mesh open and the nap relatively uncoated, and drying the fabric so that in the finished product the said fibres are covered with only a thin rubber film leaving the mesh open.

5. The process which comprises applying to a fabric a coating of substantially inert dust, then applying thereto an aqueous suspension of pre-vulcanized rubber, then washing off a part of the aqueous suspension of rubber to leave only a thin film on the fibres leaving the mesh open and the nap relatively uncoated, and drying the fabric so that in the finished product the said fibres are covered with only a thin rubber film leaving the mesh open.

6. The process which comprises applying to a fabric a coating of dust of plaster of Paris, then applying thereto an aqueous suspension of pre-vulcanized rubber, then washing off a part of the aqueous suspension of rubber to leave only a thin film on the fibres leaving the mesh open and the nap relatively uncoated, and drying the fabric so that in the finished product the said fibres are covered with only a thin rubber film leaving the mesh open. 45

ALAN E. MURRAY.